

July 20, 1943.

J. K. DUNCAN ET AL

**2,324,916**

## REINFORCED STRUCTURAL ELEMENT

Filed May 2, 1940



## UNITED STATES PATENT OFFICE

2,324,916

## REINFORCED STRUCTURAL ELEMENT

James K. Duncan, Chicago, Ill., and George L. Phelps, Tempe, Ariz., assignors to United States Gypsum Company, Chicago, Ill., a corporation of Illinois

Application May 2, 1940, Serial No. 333,006

6 Claims. (Cl. 72—38)

This invention relates to a structural element and more particularly to prefabricated reinforced cementitious units for use in building structures. The units for which this invention is especially adapted are tiles, slabs, and the like, substantially flat cementitious elements having an appreciable thickness. Sheets of this type are preferably made of gypsum or other suitable material, and are commonly used as structural floor slabs in buildings of comparatively light load occupancy and are also used as roof slabs in buildings of any type. Each tile is ordinarily provided with a tongue and groove or the like on opposite side edges and usually also with a tongue or groove on each end.

There are at present two general types of such tile in use; that is, a metal edge tile in which the slab itself is reinforced only sufficiently to hold the gypsum together and to transfer applied loads to the interlocking metal edges, which later form an I-beam, and transfer all loads to the structural framing of the building. Another type is the integrally reinforced tile which are reinforced in both directions and transfer the applied loads directly to the building framework.

Slabs of the metal edge type have a serious objectionable characteristic in their inability to support appreciable loads concentrated upon the main body of the tile. Furthermore, the insulating efficiency of the metal edge tiles is low for the reason that metal extends continuously from one surface to the other and heat is, therefore, rapidly transferred.

Tiles of the integrally reinforced type are also primarily objectionable because the edges are easily chipped, the finished tile is of low strength, and the production costs are high. In order to provide a tile of even mediocre strength, it has heretofore been found necessary to employ welded wire mesh as a reinforcing agent. This, however, has made the cost of such tile almost prohibitive.

Attempts have been made to produce a satisfactory tile using expanded metal as a reinforcing agent, since, with expanded metal as a reinforcing agent, the tile is relatively inexpensive to manufacture. Efforts in this direction, however, have been futile, due to the fact that, when manufactured in the ordinary manner, the edges of the diamonds of the expanded metal will shear the gypsum keys extending therethrough in areas near the point of application of the load and, when the gypsum keys are severed, the expanded metal mat is free to stretch in these areas and immediate failure of the tile occurs.

The present invention overcomes the previously noted objections to reinforced tile, and it is an object to provide an inexpensive, structurally strong, cementitious building unit in the form of a tile or the like, in which the gypsum keys formed through the mesh of expanded metal reinforcement will not shear or fracture under any ordinary loads applied to the tile.

Another object of the invention is to provide a reinforced cementitious unit for building structures with edges and corners which are highly resistant to chipping and abrasion.

The present invention also contemplates the production of a reinforced cementitious tile in which the reinforcement may be of expanded metal so positioned within the tile as to provide definite structural advantages and also in which the composition of the cementitious mixture is such as to effectively prevent shearing of the keys extending through the diamonds of the expanded metal.

A further object is the provision of a reinforced cementitious building unit or tile having a reinforcing member such as flat expanded metal or other suitable foraminous sheet material not under tension and in which the body of the tile is formed of a cementitious material such as gypsum or the like containing predetermined percentages of fiber, such, for instance, as ground fluff newsprint or the like.

A further object is the provision of structural units or elements comprising an aggregate containing a predetermined proportion of resilient and yieldable fibrous material whereby the elements are highly resistant to cracking strains and have other shockproof qualities which make them particularly desirable for use in earthquake-proof constructions and especially suitable for use in areas where earth tremors are prevalent.

Another object is to provide a new and novel process for manufacturing a highly shock and strainproof cementitious building unit of the character described.

45 Further objects will be apparent from the specification and the appended claims.

In the drawing:

Fig. 1 is a perspective sectional view of a tile or slab and illustrates one embodiment of the invention.

Fig. 2 is an enlarged sectional elevation of an edge portion of the embodiment illustrated in Fig. 1.

Fig. 3 is a fragmentary detail sectional view 55 taken on a line substantially corresponding to

line 3—3 of Fig. 1 and illustrates in section the keys which extend through the diamonds of the expanded metal reinforcement.

Referring to the drawing in details, the embodiment illustrated comprises a cementitious tile or slab 1 having a tongue 2 along at least one edge and a groove 3 in the opposite edge. The tile 1 is preferably formed of an aggregate comprising gypsum and a predetermined amount of fibrous material of a type and in proportions which will later be described. However, it should be understood that the tile may be formed of any cementitious material which is suitable for use in structural units and which may properly be used in connection with the fibrous material specified. Also the units may be of any desired size and shape and are not to be limited to tile.

The slab or tile element disclosed is provided with a reinforcement 4 of foraminous sheet-like material, preferably flattened expanded metal having reasonably large apertures or so-called diamonds 5, as shown in Fig. 3. In actual practice, a satisfactory reinforcement for ordinary tile may be made of standard flattened thirteen-gauge expanded metal having three-fourths inch diamonds.

The reinforcing element 4 is preferably made in the form of an elongated hollow framework such as illustrated by the dotted lines 4 in Fig. 1 and which is of a cross sectional contour approximating that of the finished slab but with depressed sides, as shown at 6, so that, when the complete slab is formed, the sides 6 are spaced somewhat from the flat sides 7 of the tile. The reinforcing expanded metal mat is also so formed that it is substantially at the surface of the slab adjacent the edges 8 and around the tongue 2 and all of the adjacent corners. The reinforcing mat is also formed at the opposite edge so that it is substantially at the surface of the groove 3 and the adjacent edges and corners as shown. The mat extends closely adjacent the surface of the tile for an appreciable distance along the flat sides thereof, as indicated at 9. By this means, a tile may be formed which is exceptionally resistant to chipping and abrasion of the tongue and groove and all adjacent surfaces and corners.

The exact areas at which the reinforcing is at or near the surface may, of course, be varied, and, in fact, the reinforcement may not be completely coextensive with the entire areas of the tongue and groove. Also the exact proximity of the reinforcing element to the surface of the tile in the vicinity of the edges and in the vicinity of the tongue and groove may be varied somewhat. For instance, in Fig. 1 the reinforcement adjacent the edges is shown just slightly under the surface of the cementitious material, and at the sides 6 it is very materially spaced from the outer surfaces 7 of the tile. Fig. 2 illustrates substantially the same reinforcement. However, in Fig. 2 the reinforcement in the tongue and groove and at the edge surfaces is shown substantially flush with the surface of the tile.

It will, of course, be obvious that reinforcing elements shaped in accordance with the disclosure herein may be employed in building units formed from any suitable cementitious material. However, particularly desirable and unexpected characteristics are obtained in the finished product when the aggregate from which the tile is formed is made with certain predetermined proportions of cementitious material and fiber in

combination with the specified type of reinforcement.

It is desirable not to have the main body of the reinforcing material (that is, the sides 6 thereof) too closely approach the surface at the sides of the tile or panel. By spacing the reinforcement substantially as shown, the diamonds are engaged by well formed efficient keys 9, as in Fig. 3, with a suitable amount of key-supporting material on each side of the expanded metal.

A satisfactory process for forming the structural unit disclosed or its equivalent consists in preparing a mold of the desired size and shape, greasing the inner surfaces of the mold, placing therein an expanded metal reinforcing element 4 of the formation described, that is, of a shape approximating the unit and with depressed sides as shown, then filling the mold with a cementitious slurry comprising stucco and fiber in the amount of 2½% to 14% by weight of the dry stucco and water in a quantity sufficient to yield a consistency of between 60 and 80. This cementitious slurry is poured into the mold containing the reinforcing element and then allowed to set. If it is desired that the reinforcing element should be slightly under the surface at the tongue and groove and adjacent edges of the finished product, then the reinforcing element may be supported in the mold accordingly. If, however, it is desired that the reinforcing element should be at the surface at these points, then it may be supported directly by the mold itself.

While the slurry composition above specified (that is, containing 2½% to 14% of the fiber by weight of the dry stucco) is satisfactory under certain conditions, it has been found that, to obtain the most satisfactory results, the fiber should be in the amount of 4% to 6% of the dry stucco. It has also been found that, for the average tile, three-fourths inch thirteen-gauge flattened expanded metal used as a reinforcing medium provides a most satisfactory product. In other words, the combination of a cementitious mixture having a relatively high fiber content with flattened expanded metal reinforcement produces a tile with remarkably efficient and unexpected characteristics.

Heretofore it has been the practice to admix comparatively small amounts of fiber (up to 1% or 1½% by weight) with the stucco in the manufacture of cementitious tile, the object being to increase the bond of the tile and reduce its density somewhat. In so far as known, however, there has never been any relationship of the proportion of fiber used to a reinforcing element of any type. In the development of the present invention it has been found that, by increasing the fiber content to from 2½% to 14% by weight of the stucco, and preferably to from 4% to 6%, and using expanded metal, and particularly flattened expanded metal, as the reinforcing agent, it is possible to produce an excellent tile having greater load-supporting characteristics and less chipping and breaking of corners and edges than any similar tile heretofore produced.

It has also been found that, when ordinary unflattened expanded metal is used, a relatively high proportion of fiber must be used to produce satisfactory results. However, if flattened expanded metal reinforcement is used, satisfactory tile may be made with a somewhat lower fiber content. In other words, there is a direct relationship between the proportionate amount of fiber and the type of reinforcement used.

As previously stated, the results accomplished by the combinations used in this invention have been very unexpected and, although it is desired that the invention should not be limited by the following theory, it is thought that the explanation for the surprising results obtained is substantially as follows:

With ordinary unflattened expanded metal employed in a tile made from a standard mix containing substantially 1% to 1½% of fiber, there is practically no "give" of the stucco when the strands of the expanded metal press severely against the gypsum keys by reason of a load being applied to the tile in that vicinity. The expanded metal, being unflattened, does not develop its full strength at the first stretch, but tends to stretch until it has been pulled into a flattened condition. The result is that, with a very heavy load concentrated on the tile, the strands of the unflattened expanded metal move sufficiently to break the nonresilient stucco keys, thereby causing complete failure of the tile. By preflattening the expanded metal, its initial stretching in the tile is substantially eliminated, thus enabling a tile, even if made from the ordinary stucco mix, to support any load less than that sufficient to cause movement of the strands of the flattened expanded metal. Although the flattened expanded metal, even when used with the ordinary stucco mix, yields a somewhat stronger tile than when unflattened metal is used, approximately the entire stress of the load is still borne by that portion of the reinforcement which is in the immediate vicinity of the point of application of the load.

The addition of a substantial quantity of fibers to the stucco mix conditions the mix for resilient or yielding intimate co-operation with the expanded metal so that the mix and the reinforcing metal fully co-operate to produce the most effective results. The fibers present, particularly in the stucco keys, cause the keys to be somewhat yielding and resilient, with the result that, when a concentrated stress is applied to the tile, the strands of expanded metal are permitted to move sufficiently to enable a large portion of the strain to be transmitted to other keys and other portions of the tile, thus relieving the gypsum keys in the immediate vicinity of the load to a very marked extent.

In tests made by using a stucco mix containing the standard amount of fibers with nonflattened expanded metal reinforcement, the failure of the tile has been due to the shearing of the gypsum keys in the vicinity of the point of application of the load. In tile containing substantial quantities of fiber and employing flattened expanded metal, the failure has been due to the rupture of the metal reinforcement.

The presence of substantial quantities of fibers with expanded metal reinforcement insures a considerably improved tile, even when the reinforcing expanded metal is unflattened. However, even to obtain this improvement, a fiber content of 2½% to 14% by weight of the stucco should be used, and, when fiber is used in these proportions in combination with flattened expanded metal, a much greater improvement is observed. However, if flattened expanded metal is used and a fiber content of from 4% to 6% by weight of stucco, the greatest efficiency may be obtained. It will, of course, be understood that these percentages may vary slightly, depending upon the type of fiber used, the size of the mesh of the expanded metal, and the gauge thereof.

In the manufacture of standard tile it is undesirable to have the fibers present in too large quantities for the reason that they tend to weaken the body of the tile somewhat. Therefore, in the present invention the proportion of fibers and type of reinforcement bear a definite predetermined relationship to each other. That is, by the use of flattened expanded metal reinforcement and a mix containing fiber such as ground fluff newsprint, or the like, in a predetermined amount in excess of that ordinarily used and which would otherwise be detrimental in standard tile, tile may be produced having greatly improved load bearing characteristics.

10 In addition to being an exceedingly strong structural unit which is relatively cheap to produce, tile made in accordance with this invention have a number of other important characteristics. Tests have shown that they are not nearly as subject to fatigue as are metal edge tile of similar dimensions. That is, when subjected to a continuous load over a long period of time, the amount of ultimate deflection is much less than that of metal edge tile and the amount of its deflection becomes constant considerably more quickly.

15 Another advantage which the tile of this invention has over metal edge tile and the like is its ability to support loads concentrated upon its main body. This characteristic permits the use of linoleum and the like directly over a floor of tile made in accordance with this invention without the necessity for a subfloor of a rigidity sufficient to carry loads to the edges of the tile.

20 Moreover, the tile being reinforced in all directions, the necessity for a tongue and groove on the ends of the tile is no longer present.

25 It is intended, of course, that the invention should not be limited to the specific embodiment or embodiments disclosed herein, since many modifications may be made, and it is contemplated, therefore, by the appended claims to cover any such modifications as fall within the true spirit and scope of this invention.

30 45 Having thus described this invention, what is claimed and desired to be secured by Letters Patent is:

1. A load supporting reinforced building slab or tile of set cementitious material comprising 35 stucco and fiber and an expanded metal reinforcing element embedded in said slab and substantially coextensive therewith, said reinforcing element being substantially flush with the surfaces and corners at and adjacent two opposed edges of said slab and spaced from the surface throughout the major area of both sides of said slab.

2. A reinforced building slab or tile of set cementitious material comprising stucco and fiber and an expanded metal reinforcing element embedded in said slab and substantially coextensive therewith, said reinforcing member comprising an expanded metal shell of substantially the same cross sectional contour as 50 said slab but having a major portion of each side depressed so that the depressed portions are materially spaced from the side surfaces of said slab.

3. A reinforced building slab or tile having a 55 tongue on one edge and a groove in the opposite edge, said tile being formed of set cementitious material comprising stucco and fiber and an expanded metal reinforcing element embedded in said tile, said reinforcing element being of a cross

60 sectional contour substantially conforming to 65 said tongue and groove.

the cross sectional contour of said tile and being substantially at the surface of said tile adjacent its edges including said tongue and groove, and having its sides depressed, so that major portions of said sides are spaced materially from the sides of said tile, the amount of fiber to stucco being from 2½% to 14% to provide sufficient resilience or yieldability in said material to prevent shearing or fracture of said material by said expanded metal when extreme loads are localized on said tile and to transmit localized stress to a comparatively large area of the material substantially in the plane of said reinforcing element.

4. An article of manufacture comprising a reinforced cementitious tile or slab having embedded therein a reinforcing shell of flattened expanded metal preformed to a shape and dimensions closely approximating the outer contour and dimensions of said slab adjacent the edges and at the corners thereof, but with a major portion of the sides depressed to provide a relatively narrow space between said depressed portions and the adjacent sides of said slab, the body of said slab being molded of a cementitious slurry comprising stucco, and fiber in an amount of 2½% to 14% by weight of the dry stucco.

5. A load supporting tongue and groove building slab or tile of set cementitious material comprising stucco and fiber, a tongue and groove reinforcing shell of flattened expanded metal of substantially the same general over-all dimen-

sions and contour as said slab and molded therein so that the surfaces of the tongue and groove edges of said shell and of said set cementitious material are substantially coplanar, the intermediate portions of said shell between said tongue and groove edges being embedded beneath the side surfaces of said slab.

6. A reinforced building slab or tile having a tongue on one edge and a groove in the opposite edge, said tile being formed of set cementitious material comprising stucco and ground fluff newsprint fiber and an expanded metal reinforcing element embedded in said tile, said reinforcing element being of a cross sectional contour substantially conforming to the cross sectional contour of said tile and being substantially at the surface of said tile adjacent its edges including said tongue and groove, and having its sides depressed, so that major portions of said sides are spaced materially from the sides of said tile, the amount of ground fluff newsprint fiber to stucco being from 2½% to 14% to provide sufficient resilience or yieldability in said material to prevent shearing or fracture of said material by said expanded metal when extreme loads are localized on said tile and to transmit localized stress to a comparatively large area of the material substantially in the plane of said reinforcing element.

JAMES K. DUNCAN.  
GEORGE L. PHELPS.